

Sept. 11, 1951

P. RAIBOURN

2,567,401

PROCESS OF PRODUCING COLORED PHOTOGRAPHS

Filed April 18, 1947



Inventor:  
Paul Raibourn  
by his Attorneys,  
Darby & Darby

## UNITED STATES PATENT OFFICE

2,567,401

PROCESS OF PRODUCING COLORED  
PHOTOGRAPHS

Paul Raibourn, Southport, Conn.

Application April 18, 1947, Serial No. 742,460

8 Claims. (Cl. 95—2)

1

The object of this invention is to provide an economical and relatively simple method of producing useful colored photographs from color separation negatives in a single layer emulsion film.

The detailed objects of the invention and the resulting products will be fully apparent from the following description of the invention.

This invention resides substantially in the steps and series of steps comprising the processes herein disclosed and the products thereof as defined in the appended claims.

In the single figure of the drawing, there is illustrated diagrammatically in edge elevation, by way of example, one way of carrying out the process herein disclosed.

In accordance with this invention three positive subtractive images are successively printed and developed to color in a single layer of light sensitive material of a "color blind" (blue sensitive) type. The images of the separation negatives are successively printed and developed at different depths in this emulsion by the procedure hereinafter described. The emulsion of such a film may be of the panchromatic or equivalent type sensitive either to the entire visible spectrum or to a limited portion thereof as well, as suggested above, as a color blind emulsion.

In order to accomplish the objects of this invention the layer of light sensitive material will be of such thickness as to contain three imaginary depths so to speak, of such thickness as to conveniently produce images of satisfactory color contrast by the herein disclosed methods of producing the color images plus an allowance for error in the controlled penetration of solutions, as explained below. As a more dimensional definition the emulsion layer will be of the order of thickness of the well known "Kodachrome" film plus an additional thickness providing two allowances for error, the nature of which will appear more fully hereinafter.

In accordance with this invention it will be assumed that there are available three balanced separation negatives of a scene and of desired density range such as may be obtained in a well known manner with so called Wratten A, B and C5 filters. The image in the red record negative (produced by the A filter) is printed with ultra-violet light on a sensitive film as illustrated in the drawings, that is a commercial color blind silver sensitive emulsion. The printing is effected to a sufficient depth to produce a satisfactory depth of color. The printing light may be an ultra-violet light for the purpose of limiting the

2

depth of penetration of the light into the emulsion so that substantially the upper third thereof is exposed. Those skilled in the art will also recognize that such an emulsion can be controlled also as to depth of printing by dyeing it with a dye complementary to the color of the printing light. For example, it could be dyed with Uramine in the case of a blue printing light.

The concentration of the dye will be adjusted so as to produce an image in the desired depth for the density range in the separation negatives. The printing may be done while the emulsion is still wet from the dyeing process, but in this case it must be printed optically. As those skilled in the art will understand, if the film was printed while wet the hydrogen ion concentration must be carefully determined to minimize swelling of the gelatin.

The latent image thus formed will be processed to a cyan color by means of direct or coupled development with well known developers such as are used in Kodachrome.

The silver which is deposited with the color is then removed by reducing it to silver bromide with ferricyanide-bromide solution and removing it and the undeveloped silver bromide to the depth just beyond the deepest depth of developed silver with neutral hypo solution which is controlled in its penetration. This step can be carried out by combining the reducing and bleaching solutions in which case the amount of silver halide removed is controlled by adding to the solution loading agents known for the purpose, such as glucose, sodium sulphate or glycerin. If the two solutions are used separately only penetration of the hypo solution need be controlled.

The penetration of the solution in accordance with the above is controlled so that all reduced silver is removed, with the result that the silver halide in the emulsion will be removed to a slightly greater depth than the silver. This addition depth represents one of the thickness allowances for error previously mentioned. Processing the film to cause this excess penetration is an important feature of this process in that close control of penetration depth of the solution is not necessary where this allowance is provided.

There now remains in the sensitive emulsion an upper layer containing a desired cyan image, a thin clear layer (the error allowance) and a thicker layer of sensitive silver halide emulsion representing approximately two-thirds of the emulsion depth.

The image of the green separation negative

## 3

is now printed through the cyan image either optically or by contact into the remaining sensitive silver halide emulsion. Printing is optical if the previously processed film has not been dried, or printing is by contact or optical printing if it has been dried. If the film is wet at this printing stage the hydrogen ion concentration and the swelling of the gelatin is adjusted in a well known manner to the same point as in the first printing.

The resulting green record image is developed to magenta by using well known developers for the purpose either of the coupling or direct developer type. The silver image is removed as before by means of ferricyanide and hypo solution, as described above.

There now remains in the emulsion from the emulsion face downwardly:

1. A cyan image
2. A thin clear layer
3. A magenta image
4. A thin clear layer
5. A layer of silver halide emulsion.

Of course, the ferricyanide-bromide and hypo solutions were used as in the first case by controlled penetration in depth to clear the emulsion a very small distance beyond the middle image layer.

The blue record image is printed either by direct contact or optically in the manner and under the conditions set forth for the previous images. It is then developed to yellow with well known coupling or direct developers. The silver and remaining halide is then removed as before by means of ferricyanide-bromide and hypo solutions.

The film now contains color images which will be a close representation of the original if the density matrix of the three subtractive colors formed in the development approximate the following values:

|            | Cyan | Magenta | Yellow |
|------------|------|---------|--------|
| Red.....   | 1.0  | 0       | 0      |
| Green..... | 0    | 1.0     | 0      |
| Blue.....  | 0    | 0       | 1.0    |

The silver images may be colored as desired by well known toning processes in which case the silver images will not be reduced to silver halide but will remain in each case and only the undeveloped silver halide will be removed.

As is well known, colors of such characteristics are not readily available. The density matrix of a more usual and common set of subtractive colors may be:

|            | Cyan | Magenta | Yellow |
|------------|------|---------|--------|
| Red.....   | 1.0  | 0.20    | 0.1    |
| Green..... | 0.60 | 1.0     | 0.2    |
| Blue.....  | 0.30 | 0.60    | 1.0    |

This, if printed as above would not constitute a satisfactory representation of the original scene.

This group of colors, if magenta is printed through a 60% positive mask of the red record negative and the yellow through a 60% positive mask of the green record negative and a 30% positive mask of the red record negative and the contrasts neutralized and properly reduced, would form an image which would be a

75

## 4

satisfactory representation of the original scene.

Such masks can be recorded and the negatives neutralized and reduced in the original separation negatives. Where many copies are to be made this is the preferable procedure. It is also possible to record such masks automatically in the printing of the positive images, or if desired, to effect the necessary masking by a combination of these procedures.

To produce the masks in the positive printing process the procedure is as follows: In printing with blue light it is inherent that in printing the magenta image through the cyan image printing is effected through a positive which has the density of 0.30 to the blue light. The desired additional mask of 0.30 may be obtained by using a proportional reduction procedure in accordance with well known processes to eliminate 70% of the silver from the cyan image and allow 30% to remain when the magenta image is printed. In a similar manner the yellow image may be properly masked by printing through the cyan and magenta images from which all of the silver has been removed. In this way a satisfactory color representation may be obtained.

From the above description it will be apparent to those skilled in the art that the subject matter of the invention herein disclosed is capable of being practiced with the aid of variations in the photographic processes indicated above without departing from the novel subject matter herein disclosed. I do not, therefore, desire to be strictly limited to the details included herein for purposes of illustration, but rather by the scope of the claims granted me.

What is claimed is:

1. A method of producing a three-color positive film from three-color separation negatives red, green and blue, comprising the steps of printing the red record image in a single silver halide emulsion panchromatic film to a controlled depth, developing the image thus formed to cyan, reducing the silver in that image to silver halide, dissolving it and the silver halide in the emulsion below the image for a short distance to form a thin clear layer, printing the green record image in the emulsion through the cyan image, developing this second image to magenta, reducing the silver in that image to silver halide, dissolving it and the silver halide in the emulsion below the image for a short distance to form a thin clear layer, printing the blue record image in the emulsion below the magenta image through the cyan and magenta images, developing that image to yellow, reducing the silver of that image to silver halide and dissolving it.

2. In the method of claim 1, said panchromatic emulsion being dyed a color complementary to the color of the printing light.

3. In the method of claim 1, said panchromatic emulsion being dyed yellow and said printing steps being effected with blue light.

4. In the method of claim 1, the step of proportionally reducing the silver image in the first two layers to form a positive mask for printing the yellow image therethrough.

5. In the method of claim 1, the step of proportionally reducing the silver in the cyan image to provide a positive mask through which the magenta image is printed.

6. A method of producing a multi-color positive film from color separation negatives, comprising printing the images from said negatives successively to succeeding depths in a single silver halide emulsion on a supporting backing to

produce superposed image layers, successively developing each image after printing to color and to silver, and removing the silver in each layer immediately after development of each layer to color and the silver halide to a depth beyond 5 each image layer to provide a clear gelatin layer between each pair of color image layers.

7. In the process of claim 6, controlling the removal of silver and silver halide after each development by controlled penetration to form 10 said clear layer adjacent each color image.

8. In the method of claim 6, the removal of the silver image being effected by reducing the silver to a halide and dissolving it and undeveloped silver halide to form a clear layer. 15

PAUL RAIBOURN.

**REFERENCES CITED**

The following references are of record in the file of this patent:

20

**UNITED STATES PATENTS**

| Number    | Name          | Date          |
|-----------|---------------|---------------|
| 1,697,194 | Leventhal     | Jan. 1, 1929  |
| 1,958,830 | Lierg         | May 15, 1934  |
| 1,966,330 | Burwell       | July 10, 1934 |
| 1,969,469 | Mannes et al. | Aug. 7, 1934  |
| 2,059,884 | Mannes et al. | Nov. 3, 1936  |
| 2,059,887 | Mannes et al. | Nov. 3, 1936  |
| 2,113,329 | Mannes et al. | Apr. 5, 1938  |
| 2,159,600 | Murray et al. | May 23, 1939  |
| 2,186,054 | Weaver        | Jan. 9, 1940  |
| 2,200,018 | Bertrand      | May 7, 1940   |
| 2,381,234 | Symmes        | Aug. 7, 1945  |

**FOREIGN PATENTS**

| Country       | Date         |
|---------------|--------------|
| Great Britain | Aug. 8, 1939 |